

March 20, 1945.

A. BEERBOWER ET AL

2,372,052

LUBRICANTS

Filed Oct. 7, 1942



Alan Beerbower Inventor  
John C Zimmer Inventor

By P. Young Attorney

## UNITED STATES PATENT OFFICE

2,372,052

## LUBRICANTS

Alan Beerbower, Westfield, and John C. Zimmer,  
Union, N. J., assignors to Standard Oil Development Company, a corporation of Delaware

Application October 7, 1942, Serial No. 461,114

8 Claims. (Cl. 252—35)

This invention relates to an improved process and apparatus for manufacturing lubricating greases, especially aluminum soap greases. The invention is particularly adapted for continuous manufacture of such greases.

Many different attempts have been made to develop satisfactory continuous processes for manufacturing lubricating greases, but few of these methods have met with the desired degree of success, particularly due to difficulties which characterize the manufacture of certain types of greases, especially aluminum grease, and in certain respects soda, barium and lithium greases. One object of the present invention is to overcome these various difficulties of the prior art and to provide a process for the continuous manufacture of aluminum soap grease, as well as soda soap grease and even other soap greases, if desired, in simple and relatively fool-proof equipment which in operation results in a high quality homogeneous uniform and reproducible product at relatively low cost.

Broadly, the invention comprises mixing a soap and a lubricating oil at a temperature considerably below the maximum grease-cooking temperature to form a lump-free slurry, diluting said slurry with additional oil to give the proportions of soap and oil desired in the finished grease, mixing said materials to make a substantially homogeneous mixture, then passing the mixture through a heating zone of relatively large heating surface per volume, in order to get complete solution of the soap in oil with once-through operation, and cooling the resultant grease stock at least to a grease structure-forming temperature. The invention may be exemplified by mixing a dry aluminum stearate powder with oil in a sufficient amount to make a thick slurry, this mixing being preferably done in a roller or pug mill which breaks up lumps efficiently, although it may be done with an agitator in a barrel, then adding more oil, still without any substantial heating of the mass, mixing these materials thoroughly and passing them through a pipe coil heater to bring the mixture up to a suitable grease-cooking temperature, such as 250—350° F. for an aluminum soap grease, or higher for other soaps such as soda or lithium or barium, then passing the materials to a surge tank from which accumulated vapors may be discharged, and finally cooling the mixture in a suitable manner to permit the formation of the desired grease structure. Usually in the past with aluminum soap grease this cooling has been generally effected by pouring the grease stock into a large number of relatively small shallow

pans and allowing them to cool for a day or two, then returning to the kettle working the product to a uniform consistency and then packaging.

The preferred method is to pass the grease stock through a helical blade (or screw conveyor) chiller, preferably one cooling down to the transition temperature of the grease, and allowing it to remain there for the required transition period of a 1/4 hour to six hours or so, or slowly cooling the grease even on down past the transition temperature and allowing the grease to go through its final transition stages in a storage kettle or shipping containers. This procedure does not require floor space for storage and use of pans, eliminates labor, shortens manufacturing time and produces greases of uniform and satisfactory consistency from lot to lot, since the cooling operation can be more closely controlled. Pan operation, where cooling is not controlled, frequently yields non-uniform products from pan to pan.

Instead of using aluminum stearate, other aluminum soaps may be used such as aluminum naphthenate or aluminum soaps of other carboxylic acids having 10, or preferably 15, carbon atoms or more, such as aluminum soaps of synthetic fatty acids derived from the oxidation of paraffin wax, or mixtures of these various soaps, such as a mixture containing about 90% to 95% of aluminum stearate and 10% to 5% of aluminum naphthenate. Naphthenic acid or some other suitable high molecular weight acid such as oleic acid, etc., alcohols, glycols, glycerine esters, phenols, aliphatic or alkyl aryl amines or alkanolamines may be used alone or with aluminum naphthenate to modify the grease structure or change the rubbery liquid to solid gel transition temperature range attendant upon the use of aluminum stearate.

The oil to be used both in making the original slurry and in subsequently diluting the slurry to the desired final proportion of oil in the finished grease may be any of the conventionally used lubricating base stocks, such as various light, medium or heavy lubricating oil distillates or residual fractions which may have been subjected to any of the conventional refining treatments such as clay-treating, acid-treating, solvent extraction, etc., and may be derived from various crude oils such as paraffinic, naphthenic, or mixed base crudes. In addition, other suitable fluid lubricants, fuels or liquids may be compounded with soap to yield pastes, solid fuels, etc.

The proportions in which the soap and oil should be mixed in order to make the slurry in

the first step according to this invention, should be about 15 to 35% by weight of soap and 65 to 85% of oil, depending largely upon the viscosity and other characteristics of the oil used as well as the type of soap used.

Although the soap, aluminum, lithium soda, or other metal soap, which is preferably in the form of a dry powder, may be mixed with the oil in this first step without the use of any heat whatsoever, it is possible if desired to use oil which has been warmed slightly, e. g., up to 100° or 150° F., or so, to facilitate the mixing.

As suggested above, the slurry mixer should preferably be an efficient lump-breaking mixer, such as the usual roller mill, in which the periphery of a roller having a horizontal axis and a peripheral edge of substantial width, rolls in contact with the upper side of a disc roller rotating on a vertical axis, so that lumps in the material being mixed are crushed between the rollers. Other types of slurry mixers may be used such as a small grease kettle with rotating paddle blades, a bread-dough type of mixer or a parallel-roll paint mill. An effective type is also available in which two interlocking rotors knead the mass together.

Of the various types of slurry mixers described above, the Lancaster roller mill is preferred. This is described briefly as follows: The mixer tank rotates about one axis and the mixer blades about another eccentric to the first. The blades consist of both "plows" to lift the mass and "mullers" to force it against the tank bottom.

The mixer in which the slurry is subsequently mixed or diluted with more oil, which for the sake of clarity may be referred to as the blending mixer, is preferably one which is suitable for continuous operation, such as the orifice mixer. Other types of blending mixers may be used, however, such as gear or rotor pumps, in which controlled amounts of the slurry and oil are fed in together and rapidly mixed and discharged in a continuous operation, the amount of recycling of the material through the gear being controlled at will. A centrifugal pump or a rotary mixer of the colloid mill type or the Lancaster disperser type may also be used.

The heater through which the blend of slurry and oil is then passed should preferably be a pipe coil heater having sufficient inside pipe diameter to give the desired capacity, and of sufficient pipe length to give the required heating in a once-through operation. The surface of the pipe coil heater should be at least 4 square inches per cubic inch of volume and the temperature of the grease at the outlet should be between the approximate limits of 200° and 500° F., depending upon the type of grease being produced, for instance about 250° to 350° F. for aluminum, magnesium or barium soap, preferably about 280° to 300° F., and on the other hand about 350° to 500° F. for sodium or lithium soap grease, and about 200° to 250° F. for calcium, lead or zinc soap grease. Other types of heaters suitable for continuous operation are those containing a rotating scraper to insure good heat transfer, or a tube bank variety.

On the other hand, for batch operation an ordinary kettle without wall scrapers is suitable either for use with high pressure steam or heated by direct firing.

Although the surge tank mentioned above is not necessary in all cases, it is a desirable accessory in the equipment in order to provide for

venting of accumulating gases and vapors, and also in order to even out any irregularities in the volume of flow of the materials in the various parts of the equipment before or after the surge tank.

If it is desired to cool the grease, this is preferably done in a screw conveyor type of cooler, such as the Carbondale scraped chiller. If desired, of course, other types of coolers can be used such as a tubular heat exchanger or a jacketed kettle or drum with cooling water circulating through a jacket.

A standing or storage kettle may also be used, if desired, either to permit the fresh grease product to remain quiescent for a required period during which it changes from a thick solution of oil in soap and acquires the desired grease structure, or this kettle may be used merely as a temporary storage vessel.

For the production of aluminum soap greases it is desirable to use both the chiller and the standing kettle so that the hot grease may be quickly cooled down to the grease structure-forming temperature, then permitted to remain in a quiescent condition at that temperature until the desired grease structure has been acquired. If desired, two or more of these standing kettles may be used in order to provide for uninterrupted or continuous manufacture. It is also possible to discharge the grease from the chiller directly into shipping containers such as barrels, kegs or cans.

If desired, the whole equipment may be maintained and operated under a pressure slightly above atmospheric in order to prevent evaporation of water during the manufacture of a lime soap grease.

The invention will be better understood from a consideration of the accompanying drawing which shows a schematic lay-out of the equipment used in applying this invention to the manufacture of aluminum or lithium soap grease.

Referring to the drawing, aluminum soap 1, preferably in the form of a dry powder, is fed along with oil from a supply tank (not shown) through line 2 into the roller mill 3 where the soap and oil are mixed together in the form of a thick slurry and then passed by line 4 into the slurry tank 5 through slurry-metering pump 6 into line 7 where it meets oil being fed from line 2 through line 8 and oil-metering pump 9, and the mixture of slurry and oil passes from line 7 into orifice mixer 10 through line 11 into pipe coil heater 12 where the mixture is heated to the required grease blending temperature, and thence passes by line 13 into surge tank 14 and is then pumped by pump 15 through line 16 into the Carbondale chiller 17, into the standing kettle 18 where it is permitted to remain quiescent until the desired grease structure has been acquired, and finally through filter 19 and discharged into suitable containers (not shown) for shipping or storage. Suitable lines 20, 21, and 22 may be used for by-passing the surge tank 13, the chiller 17, and the kettle 18, respectively, if desired.

The advantages of this invention will be further apparent from a consideration of the following examples, showing the manufacture of an aluminum soap grease according to this invention.

#### Example 1

A blend of 33% aluminum stearate and 67% of 70 S. S. U. at 210° F. lubricating oil was mixed by hand in a beaker. This was fed through a

heating coil of copper tubing 20 feet long and  $\frac{1}{4}$ " I. D., immersed in oil at 400° F. The exit temperature was 320° F. One part of this concentrate was mixed continuously in a small centrifugal pump with 4 parts by weight of 200 S. S. U. at 210° F. lubricating oil. The final temperature was 250° F. The flow rate was about 1 lb. per minute. The stream was cooled by a steel coil 10 feet long and  $\frac{1}{4}$ " I. D., immersed in water at 180° F. On standing, a good pressure gun grease resulted.

*Example 2*

A suspension of 8% aluminum stearate in 70 S. S. U. at 210° F. lubricating oil was prepared by first mixing a concentrate of 33½% and diluting this in a kettle. This mixture was fed through a coil of 20 feet length and  $\frac{1}{2}$ " I. D., immersed in a bath of fused sodium and potassium nitrates at 400° F. The feed rate was approximately 1 lb. per minute and the exit temperature was 325° F. This melted grease was then held in a surge tank holding 15 lbs. for the transit time of approximately 15 minutes, allowing air which had been trapped in the suspension to escape. This melted, de-aerated grease was then pumped through a cooler coil immersed in running water at 125° F. The exit temperature was 150° F. and the grease was stored in containers at this temperature until set. A satisfactory cup grease was produced. Lithium, calcium, barium, lead, zinc, soda or other soap may be similarly employed to make the respective types of grease, or soaps such as soda, lithium, barium, lime, freshly prepared in a kettle or other equipment by direct saponification of fats or fatty acid with the respective alkalis may be fed directly into the mixing equipment for blending with oil cooling and the formation of greases.

This invention is not intended to be limited to the specific examples which have been given merely for the sake of illustration, but only by the appended claims in which it is intended to claim all novelty inherent in the invention as well as all modifications coming within the scope and spirit of the invention.

We claim:

1. Process for manufacturing grease which comprises mixing a soap and oil at a temperature substantially below the grease-cooking temperature to form a slurry, diluting said slurry with additional oil to give the proportions of soap and oil desired in the finished grease, mixing to make a substantially homogeneous mixture, passing said mixture to a heating zone of relatively large heating surface per volume in order to heat it to at least a grease-cooking temperature and get complete solution of the soap in oil with once-through operation, and cooling the resultant grease stock at least to a grease structure-forming temperature.

2. Process according to claim 1 in which the heating zone is a pipe coil heater.

3. Continuous process for manufacturing lubricating grease which comprises continuously mixing a soap and a mineral lubricating oil base stock in proportions to form at a temperature substantially below a grease-cooking temperature a thick, smooth relatively homogeneous slurry, mixing in grease forming proportions, quantities of slurry with additional quantities of oil, continuously passing the resultant mixture through a heating zone of relatively large heating surface per volume to heat it in one pass to at least a grease-cooking temperature, and contin-

uously passing said fresh grease stock through a surge tank to insure complete and homogeneous solution of the soap in the oil and the release of formed or entrained gases and vapors, then passing the soap oil solution through a cooling zone to form the grease structure.

4. Continuous process for the manufacture of an aluminum soap lubricating grease which comprises continuously mixing a dry aluminum soap powder and a mineral lubricating oil base stock at a temperature of below about 150° F. to form a thick, smooth relatively homogeneous slurry with about 15 to 35% by weight of aluminum soap and about 65 to 85% by weight of mineral oil mixing in controlled grease-forming proportions said slurry with additional quantities of mineral oil, continuously heating the resultant blend of slurry and oil to a temperature of about 250 to 350° F. in a heating zone of sufficiently large heating surface per volume to get complete solution of the soap in oil with once-through operation, continuously passing the resultant fresh stock through a surge tank to insure complete and homogeneous dispersion of the soap in the oil and release of formed vapors, quickly and continuously cooling the resultant mixture to a grease structure-forming temperature of about 100 to 150° F., and continuously passing said cooled mixture into one of a plurality of transition zones where said grease stock remains quiescent until it acquires the desired gelled structure, and continuously removing finished aluminum soap grease from at least one of said transition zones.

5. Process according to claim 4 in which the slurry is formed from said soap powder and oil base stock by passing through a roller mill, metering pumps are used for continuously feeding slurry and oil together into an orifice mixer, the heating is affected in pipe coil heater of at least 4 square inches of heated area per cubic inch of volume, and the hot grease stock is pumped through a helical scraped cooler.

6. Continuous process for the manufacture of a lithium soap lubricating grease which comprises continuously mixing a dry lithium-fatty acid soap powder and a mineral lubricating oil base stock at a temperature of below about 150° F. to form a thick, smooth homogeneous slurry with about 15 to 35% by weight of lithium soap and about 65 to 85% by weight of mineral oil, mixing in controlled grease-forming proportions said slurry with additional quantities of mineral oil, continuously heating the resultant blend of slurry and oil to a temperature of about 250 to 500° F. in a heating zone of sufficiently large heating surface per volume to get complete solution of the soap in oil with once-through operation, continuously passing the resultant fresh stock through a surge tank to insure complete and homogeneous dispersion of the soap in the oil and release of formed vapors, quickly and continuously cooling the resultant mixture to a grease structure-forming temperature of about 100 to 150° F., and continuously passing said cooled mixture into one of a plurality of transition zones where said grease stock remains quiescent until it acquires the desired gelled structure, and continuously removing finished lithium soap grease from at least one of said transition zones.

7. Apparatus for the manufacture of lubricating grease, which comprises a mixer adapted to break up lumps sufficiently and to make a thick homogeneous slurry, a slurry supply tank, an-

other mixer, and a heater, together with means for feeding a dry soap powder and a mineral oil into the first slurry mixer, means for passing the resultant slurry into the slurry supply tank, means for withdrawing the slurry from said slurry supply tank into the second mixer, means for feeding a mineral oil also into said second mixer, means for passing the mixture produced in said second mixer into the heater, means for withdrawing hot grease stock from said heater.

8. Apparatus according to claim 7 in which the slurry mixer is a roller mill and the second mixer is an orifice mixer, metering pumps are used as the means for feeding slurry and oil into the

orifice mixer, said apparatus also comprising a surge tank to insure complete homogeneous dispersion of the soap in the oil and the release of formed vapors, a helical scraped cooler, a pump for passing hot grease from the surge tank through said cooler, a plurality of transition zones connected in parallel and means for passing cooled grease stock from the cooler into any one of said transition zones, and means for withdrawing a finished grease stock from any one of said transition zones and discharging same through a filter.

ALAN BEERBOWER.  
JOHN C. ZIMMER.